

# UNITED STATES PATENT OFFICE.

WILLIAM A. McADAMS, OF BAY SHORE, NEW YORK.

## ALUMINUM ALLOY.

1,146,185.

Specification of Letters Patent. Patented July 13, 1915.

No Drawing.

Application filed November 14, 1914. Serial No. 872,237.

*To all whom it may concern:*

Be it known that I, WILLIAM A. McADAMS, a citizen of the United States, and resident of Bay Shore, in the county of Suffolk and State of New York, have invented 5 a new and useful Aluminum Alloy, of which the following is a specification.

My invention relates to an aluminum alloy particularly adapted to casting purposes 10 and consisting of aluminum, silver, copper and cadmium. These parts are combined substantially in the proportions of aluminum eighty-two parts by weight, silver one part, copper twelve parts and cadmium five 15 parts.

In forming the alloy, the aluminum is first melted, the copper is then added and the two melted together, then the silver is added, then the temperature is lowered as 20 low as it can be and yet remain sufficiently high to melt the cadmium when the latter is introduced, and the mixture is thoroughly stirred and then poured into molds to form the article to be cast, or into molds to form 25 ingots for shipment for further use.

It has been ascertained by a careful test of more than a year, that this alloy will withstand the action of spring or lake wa-

ter, such as is commonly distributed in city 30 water supplies, without corrosion or stain, and, while brass and bronze faucets and fixtures have been found to sweat under an internal pressure of sixty-five pounds to the square inch, the present alloy has withstood successfully two hundred pounds internal pressure to the square inch without 35 such sweating. Aside from its non-sweating and non-corrosive qualities, it is much lighter in weight than bronze or copper for shipment and handling.

What I claim is:

An aluminum alloy composed of aluminum, silver, copper and cadmium combined substantially in the proportion of eighty- 45 two parts by weight of aluminum, one part by weight of silver, twelve parts by weight of copper and five parts by weight of cadmium.

In testimony, that I claim the foregoing as my invention, I have signed my name in 50 presence of two witnesses, this 30th day of October, 1914.

WILLIAM A. McADAMS.

Witnesses:

HENRY C. THIEME,  
LIDA M. EGBERT.